

## UNITED STATES PATENT OFFICE.

CHARLES E. PARSONS, OF NEW YORK, N. Y., AND SAMUEL PEACOCK, OF WHEELING, WEST VIRGINIA, ASSIGNEES TO METAL RESEARCH CORPORATION, OF NEW YORK N. Y., A CORPORATION OF DELAWARE.

## PROCESS OF PRODUCING PURE IRON FROM ITS ORE.

No Drawing.

Application filed October 17, 1923. Serial No. 669,111.

This invention relates to a process of producing pure iron from its ore, and has for its object to improve the procedure of making the same, over what has been heretofore known.

With these and other objects in view the invention consists in the novel steps and combinations of steps constituting the process, all as will be more fully hereinafter disclosed and particularly pointed out in the claims.

The process of this invention makes pure iron by employing a temperature of reduction which does not permit the iron ore to sinter, and therefore, it does not collect impurities, such as slag, silica, etc. As is well known, should these impurities become embedded in the fused mass of the iron, the subsequent step of separating out the pure iron from the gangue would fail to remove all the impurities, and therefore, upon the later fusion of the pure iron, after passing the magnetic separator, such impurities would remain with the metal and later cause more or less metalloids to form and thus lessen the purity of the resulting product. It is also known that unless pure iron is produced above a given temperature, it will constitute when formed what is known as pyrophoric iron, which is chemically very active, and therefore, not suitable for the purposes in hand. It is therefore necessary in carrying out this process, to heat the iron oxide above 1500° F. which will prevent the presence of pyrophoric properties in the iron; and it is also necessary to so control the temperature that it will not go above 1800° F., for otherwise its purity will be decreased.

In order that the invention may be the more clearly understood it should further be said that the metallurgy of iron and steel as usually practiced at this time, consists in reducing iron oxide usually with carbon or carbon monoxide, producing a crude iron carbide and treating such crude metal by various methods to remove impurities. Such refining processes consist largely in "puddling" or kneading the crude metal to separate out the relatively low melting point impurities, or in burning with air and slag-

ging out the metalloids. All these processes are costly and are not technically effectual. The puddling process does not clear the metal of slag, but gives a product containing relatively very small quantities of occluded gases and oxidation products, nitrogen compounds, etc. The air processes of the Bessemer and open hearth type of furnace are capable of removing more or less slag and the metalloid impurities forced into the metal by the blast furnace process, but in doing so they charge the metal with dissolved gases, iron oxidation products in solid solution in definite proportions, and undetermined forms of nitrogen compounds. It is possible, it is true, with elaborate and costly refining operations, to greatly minimize the objectionable effects of these refining treatments, but a positively homogenous metal is substantially never realized, thus giving rise to an inevitable uncertainty as to the performance of such refined iron when used industrially.

By the process to be disclosed below, these objections are removed as will presently appear. Further, the so-called "pig" iron or blast furnace smelted iron varies considerably in composition, depending upon the ores and coke employed and the method of working the furnace. An approximate general analysis showing the impurities in such iron, may be stated as follows:

|                         | Per cent. |
|-------------------------|-----------|
| Iron carbide            | 55.8      |
| Iron manganese sulphide | 4.1       |
| Iron silicid            | 7.5       |
| Iron phosphide          | 1.2       |
| Iron                    | 31.4      |

All these impurities are forced into the crude metal by the nature of the blast furnace smelting, in which the ore and its accompanying impurities such as silica, and alumina are mixed with a flux to slag the silica, etc., and by the coke to supply heat. This mixture is charged into a closed system furnace such as a blast furnace, and the whole mass, exclusive of fuel carbon, is melted down together. All components of this furnace mixture, together with the necessary fuel, are charged into the furnace

as solids and can only escape as liquids or gases. As a result, very high temperatures must be employed and the furnace must be operated constantly under positively reducing conditions, and there are no practicable means of separating impurities, except by the difference in densities of the melted or gaseous products.

The carbon itself is initially burned to carbon monoxide, thus utilizing scarcely more than one third of its heating power so far as the melting zone of the furnace is concerned. Unfortunately, elemental iron readily forms compounds with metalloids, hence silicon from the silica, and carbon from the coke together with the highly objectionable sulphur and phosphorus in the furnace charge tend to ultimate in the crude iron. Iron ore generally contains very little sulphur, but the coke necessarily employed contains from one to two percent, and of the total sulphur in the furnace charge, about 90% comes from coke. This sulphur must be as completely removed as possible, and this is usually done by adding a relatively large proportion of lime to the furnace charge, which requires still more coke for its conversion to a fusible slag, so that at best, sulphur elimination is never more than partial. By the procedure of this invention, these objections are likewise eliminated as will presently appear.

In addition to the foregoing objections, the fuel proportion is greatly augmented, under the prior procedures, because to form and melt a pound of slag requires seven times as much coke as is necessary to reduce from the oxide and melt a pound of iron. The inefficiency of the blast furnace process is indicated by the fact that while somewhat less than one third of a pound of coke is technically sufficient to reduce and melt a pound of iron from iron oxide, more than one pound is required in actual practice and the result is a very crude iron product of minor industrial value, unless it is further refined.

These last named objections are likewise obviated by the procedure disclosed below. Again, although pig iron refined by the kneading or puddling process gives a moderately uniform product, yet, the operation is entirely too costly for general industrial application. And the Bessemer and open hearth processes, while almost universally employed, give a very uncertain product. In fact, Sir Roberts Austin experimentally determined that steel made by such methods, contains from six to eight times its volume of gases which high temperatures alone will not remove, and ample evidence supports the belief that these dissolved gases are seriously objectionable, although elaborate and costly processes have been devised for their removal as an industrial pro-

cedure. It results that most of these methods involve adding further impurities, and none of them are positive in effect. Also in these smelting processes, from the blast furnace through the open hearth furnaces or converters, a considerable proportion of rejected materials are produced, which generally contain too much iron to discard as waste and which must be reworked in the blast furnace. In fact, it is safe to say that practically over 25% of the total iron smelted in a blast furnace connected with steel making is reworked metal which must bear again and again the cost and losses of smelting.

The process of this invention again avoids these objections as will appear more fully hereinafter.

According to this invention, on the other hand, pure iron may be produced direct from the ore by the following procedure which consists simply in reducing iron oxide at about 1500° F. in a stream of reducing gas which has previously been desulphurized by any suitable means. The gas which may be derived from coal or oil, or by the well known producer gas, is used in excess, and after passing through the reducing chamber, is further utilized as fuel. By this means, iron oxide is reduced to metallic iron at so low a temperature that no slag is formed, no sulphides or phosphides are made, nor are any metalloids reduced to elemental form. The reduction must be effected in a closed system with a large excess of reducing gases flowing in a counter current to the movement of the ore. By using the reducing gases in excess and maintaining in the reducing chamber a partial pressure of carbon dioxide, or water vapor, never in excess of 5 centimeters, practically a quantitative reduction of iron oxide may be realized. The ore prior to reduction is thoroughly dried and passed through rolls to evenly size the particles of mineral and prevent clumping.

It is not practicable to completely reduce ferric oxide, or the magnetic oxide with a theoretical quantity of carbon monoxide only in the presence of the catalytically reacting pyrophoric elemental iron in contact with carbon monoxide, because there will result the following reaction:—



This reaction is strongly exothermic, yielding, in fact, 1240 B. t. u. per pound of carbon monoxide reduced. No great concentration of carbon dioxide is possible owing to the presence of elemental iron in excess, but this reaction will deposit carbon on the metal, pyrophoric metal, if present, and it would be difficult to later remove it.

But, if once deposited and not removed, the carbon would ultimate as iron carbide when

the iron is melted thus destroying its purity. Above 1200° F., however, the carbon deposition reaction velocity from the gas is greatly reduced and at about 1400° F. a revision of the pyrophoric properties of the iron commences. But there is always possible, a momentary temperature drop which may deposit carbon upon the reduced pyrophoric metal and thus upon fusion, introduce iron carbide into the end product of iron. But, this is avoided by providing in the apparatus a positive temperature control which prevents the iron from reaching a point below a predetermined degree. Probably equally undesirable is the presence of a small, even minute quantity of ferrous oxide which may accompany the carbon deposition, and which would dissolve into the iron upon fusion. Therefore, to avoid these objections the temperature ranges employed must be strictly maintained within narrow limits not above 1800° F. and not below 1500° F.

Coal gas may be used as a reducing agent containing about 47% hydrogen. A gas of this type contains by volume approximately:

|                               |       |
|-------------------------------|-------|
| CO                            | = 8%  |
| CO <sub>2</sub>               | = 3%  |
| CH <sub>4</sub>               | = 32% |
| C <sub>2</sub> H <sub>4</sub> | = 5%  |
| H <sub>2</sub>                | = 47% |
| N <sub>2</sub>                | = 4%  |

The gas and ore are preheated to any desired temperature. By this means, the ore and reducing agents may be kept above the temperature at which pyrophoric iron can exist and at which the CO can deposit carbon.

If hydrogen is used as a reducing agent, the reaction is strongly endothermic requiring about 347 B. t. u. per pound of iron thus formed, and allowance is made for such heat. The heat produced by reducing ferric oxide with carbon monoxide at 1500° F. amounts to about 139 B. t. u. per pound of iron thus made, and does not constitute a thermal obstacle to the process.

Average Lake Superior iron ore has approximately the following composition:

|                    | Per cent. |
|--------------------|-----------|
| Elemental iron     | 56.8      |
| Ferric oxide       | 81.2      |
| Silicia            | 8.3       |
| Alumina            | 2.5       |
| Lime phosphate     | .4        |
| Lime sulphate      | .1        |
| Lime carbonate     | .3        |
| Magnesia carbonate | .4        |
| Manganese dioxide  | 1.2       |
| Volatile matter    | 5.6       |

The iron oxide of this ore may be separated out by an oil separation, or by other well known ore treating operations, produc-

ing as an end product, iron oxide of a purity exceeding 99.9%; or the crude iron oxide may be reduced to elemental iron, and such iron removed from the gangue material by a magnetic separation.

70

After treatment with reducing gas, as described above, if crude ore is employed, there remains in the solid form from 100 pounds of such ore, 56 pounds of elemental iron and 14 pounds of gangue material, the latter having passed through the reducing chamber unchanged. The solid matter is conveyed out of the reducing chamber by any suitable means, and, after cooling below the magnetic transformation point or substantially below 1400° F. is passed through a magnetic separator by means of which, in two or more passes, the elemental iron is completely separated from the gangue matter and is physically in the form of a fine powder and substantially chemically pure as it has not been in contact with carbon or metalloid oxides at a higher temperature than about 1500° F. The iron powder is then suitably delivered into an electric furnace of the induction or similar type, by means of which it is melted into a mass without contact with carbon electrodes, or in any way subjected to carbonaceous material. The molten product is pure iron.

90

95

Its positive freedom from gaseous occlusions, metalloid solutions and slag inclusions of any kind preclude the presence of alloy eutectics or eutectoids, and constitutes this metal as a composition or state of matter never heretofore known in mass as an industrial product.

100

Its industrial usefulness is wide and varied; it has a low corrosion factor, is easily worked without strain hardening, and may be shaped as readily as zinc or tin. Its chief use, however, is in making steels free of gaseous occlusions and metalloid eutectoids.

105

For such purposes it is only necessary that a suitable alloying metal or compound be added in the desired proportions to the molten pure iron. Any desired alloy effect may be positively and exactly duplicated at will, an accomplishment quite impossible under the present method of making special steels.

110

For making straight iron carbides for carburizing iron and steel without adding impurities, this metal, brought to a high temperature such as 4000° F. in contact with pure carbon will take up nearly 10% of carbon. An alloy of iron and carbon of this nature enables the manufacturer to produce a wide range of iron carbon steels of exceptional purity and of positive physical properties. There can be no blow holes in an ingot made of such materials, and practically no lamination or segregations in the worked metal.

120

125

It will now be clear that by following this process, iron oxide is reduced by means of

130

a reducing gas, at a low temperature. Illustrating with carbon monoxide and with hydrogen, the reactions may be stated thus:—



For every pound of iron reduced with carbon monoxide, 139 B. t. u. are liberated; reduced with hydrogen; 347 B. t. u. disappear. As the reaction product for the manufacture of one pound of pure iron with carbon monoxide, consists solely of one and one-fifth pounds of carbon dioxide, assuming a radiation loss of 15%, producing iron by this means is a heating effect and must be supplied in the heating chamber to regulate the combustion of the gases used for heating the charge, to avoid too high temperatures. If the hydrogen is employed as the reduction reagent, heat is absorbed and there is no danger of objectionably high temperatures in the reducing chamber.

According to the theory of allotropy, all allotropic substances are complex, and if ferric oxide is reduced at a temperature different from that at which the oxide was formed originally, a metallic phase different from the original metallic state will be obtained. When iron oxide is reduced very slowly at about 750° F. the elemental iron thus obtained, has very different physical properties from those of ordinary iron at 750° F. The elemental iron produced at such low temperature consists possibly of ferrous ions exclusively, and constitutes substantially the state of iron usually known as pyrophoric. Pyrophoric iron is extremely active, as above stated, and its presence in elemental iron produced by gaseous reducing reagents, very markedly lowers the efficiency of reduction, because the partial pressure proportion of the gaseous reaction product is enormously reduced. That is, the reaction reverses at vastly lower partial pressures of carbon dioxide or water vapor than is usually observed in studying reactions with ordinary iron. This, of course, seriously involves the commercial application of reducing pure iron by gaseous reducing agents; and means must be found for the elimination of the pyrophoric state in such reduced elemental iron.

In fact, pyrophoric iron maintained at 600° F. for 48 hours, loses most of its "active" tendency, and at 650° F. for 24 hours, the pyrophoric state entirely disappears; but, holding a charge of such iron for 24 hours under narrow temperature limits, is a difficult and costly industrial operation.

The general proposition has been confirmed that the well known iron alpha-beta transformation point, about 1420° F. (770 C.), is not an ordinary transition phenomenon, and that at such temperature, an inner equilibrium is established with great veloc-

ity; and that above such transition point, pyrophoric iron does not exist. It is essential to this process, therefore, that at all stages of the reducing operation the temperature of the elemental iron shall never fall below 1500° F. as produced; and to avoid sintering and thereby entangling particles of gangue matter in such manner as to cause the magnetic separation to fail, the reducing temperature must not exceed 1800° F.

Pure ferric oxide melts at 2854° F. and sinters readily at 2300° F. The crude oxide as it occurs in iron ore, sinters appreciably at 1850° F. Therefore, for efficiency in the operation of our process, the iron oxide under treatment in the reducing phase should never fall below 1500° F. nor exceed 1800° F.; also in drying the ore and driving out water and organic matter, the maximum temperature employed should not exceed 1800° F.

It is obvious that after reduction to elemental iron the material must be cooled below the magnetic transition point, 1420° F. in order to enable magnetic separation. The cooling of the finely divided elemental iron under such conditions does not restore the pyrophoric state. As a further means of preventing the formation of pyrophoric iron, thus enabling quantitative reduction of iron oxide at low temperatures, a negative catalyst may be mixed with the oxide, such as arsenic acid in very small proportion; or a few hundredths of one percent of chlorine may be added to the reducing gases. While such practice enables lowering the temperature of reduction, it does not enable the use of temperatures higher than 1800° F. in the preparatory stages.

In the practical operation of our process, the iron oxide is thoroughly dried and organic matter burned out, when present. The ore is then passed through a reducing apparatus, the temperature being positively maintained between 1520° and 1800° F. The reducing apparatus may conveniently consist of the well known constructions to which no claim is made but involving three or more reducing decks upon which the ore is slowly delivered at a point on the outer circumference of the uppermost deck. Revolving arms having plow shaped stirrers attached, slowly move the ore in successive circular ridges, from the circumference of the deck to a central aperture, when the charge falls to the deck below. On this deck the plows attached to the revolving arms, work the charge in successive ridges to the circumference of the deck, where apertures suitably placed, enable the ore to fall to the next lower deck; this treatment of successive ridging is continued on as many decks as the particular ore under treatment may require. One or more upper chambers may be used

for heating the ore when required, by burning a portion of the reducing gases within such chamber or chambers. The reducing gases enter the reducing furnace at the bottom deck and pass through and over the successive decks, in counter current to the flow of the furnace charge. The discharge from the reducing furnace, passes over magnetic separators to eliminate gangue, and the pure iron powder is discharged into an induction furnace for fusion. The whole system, from the reducing furnace to the induction melting furnace is sealed in a closed system.

The performance of the reducing furnace is the controlling factor in the process. It is known that the efficiency of deoxidation of iron oxides by means of reducing gases is less a function of fineness of subdivision than of surface contact between the oxide and the reducing reagent. By means of a plow stirring effect, fresh surfaces are constantly being exposed to gas contact.

What is claimed is:—

1. The process of making substantially pure iron directly from iron oxide which consists in reducing said oxide free from carbonaceous material in the presence of a stream of sulphur free reducing gas at a temperature between 1500° F. and 1800° F.

2. The process of making pure iron directly from iron oxide ore free from carbonaceous material which consists in subjecting said ore to a stream sulphur free reducing gas in excess at a temperature above 1500° F. and below 1800° F.

3. The process of making pure iron directly from its ore which consists in subjecting said ore free from solid carbon to the action of a sulphur free stream of pro-

ducer gas at a temperature between 1500° 40 F. and 1800° F.

4. The process of making substantially pure iron directly from iron oxide which consists in reducing said oxide while in motion in the presence of a stream of reducing gas flowing in a direction opposite to the movement of said ore, said gas being free from sulphur and at a temperature sufficient to prevent the formation of iron carbide. 45

5. The process of making pure iron directly from iron oxide ore which consists in subjecting said ore to a stream of a reducing gas in excess at a temperature sufficient to prevent the deposition of carbon, and preventing the partial pressure of any carbon dioxide or water vapor that may be present from exceeding five centimeters of mercury. 50

6. The process of making pure iron directly from iron oxide ore which consists in subjecting said ore to a stream of a reducing gas free from sulphur and in excess at a temperature sufficient to prevent the deposition of carbon, and positively maintaining said temperature throughout the period of reduction. 60

7. The process of making pure iron directly from iron oxide ore which consists in subjecting said ore mixed with a negative catalyst to a stream of a reducing gas in excess at a temperature sufficient to prevent the deposition of carbon. 70

In testimony whereof we affix our signatures.

CHARLES E. PARSONS.  
SAMUEL PEACOCK.